

Sept. 22, 1925.

1,554,616

P. A. E. ARMSTRONG

HOLLOW DRILL ROD AND PROCESS OF MAKING

Filed Dec. 8, 1922



INVENTOR  
Percy A. E. Armstrong.  
BY *H. H. Dyke*  
ATTORNEY

Patented Sept. 22, 1925.

1,554,616

# UNITED STATES PATENT OFFICE.

PERCY A. E. ARMSTRONG, OF LOUDONVILLE, NEW YORK, ASSIGNOR TO LUDLUM STEEL COMPANY, OF WATERVLIET, NEW YORK, A CORPORATION OF NEW JERSEY.

## HOLLOW DRILL ROD AND PROCESS OF MAKING.

Application filed December 8, 1922. Serial No. 605,699.

*To all whom it may concern:*

Be it known that I, Percy A. E. Armstrong, a subject of the King of Great Britain, and a resident of Loudonville, county of Albany and State of New York, have invented a certain new and useful Improvement in Hollow Drill Rods and Processes of Making, of which the following is a specification.

10 Part of the subject matter of the present application is divided out of my prior application Serial No. 318,253, filed Aug. 18, 1919, and another part is taken from my prior application Serial No. 528,753, filed 15 Jan. 12, 1922.

According to the present invention, the drill rod or similar tubular body is rolled down from an ingot having its bore formed by casting around a tube, which tube becomes welded in place in the casting or casting and rolling operations, forming an integral part of the ingot and drill rod; and this tube is filled with material, such as sand, prior to the casting operation, the 20 original sand core remaining in place during the rolling operation, as well as the casting operation, and being finally removed from the completed drill rod. The term "sand" is used for convenience to include 25 materials non-frittable under high heat, such as sand, finely divided burnt magnesite, talc, flint shot, and the like.

The tube is preferably of mild or low carbon steel and the remainder of the ingot 30 and drill rod of hard or higher carbon steel, and either or both may contain suitable additions of alloying materials, if desired. The mild steel of the tube, while absorbing additional carbon by saturation from the 35 surrounding cast steel, remains relatively tough and serves to strengthen the drills and to prevent cracks in the drills forming or beginning at the bore thereof.

It is of great importance in connection 40 with this invention that the sand filling of the tube remain in place from the commencement of the fabrication until the completion thereof. The bore of the tube is preferably cleaned of all oxides, as by pickling, so as to present a clean metallic surface, and the filling material, designated for 45 convenience as sand, is likewise clean and free from oxides, such as iron rust. In this way I am enabled to obtain the necessary 50 bore in a very simple, convenient and accu-

rate way, to carry out the various operations without intermediate interruptions, as for filling the tube with sand after casting the ingot, and the oxides, etc., which would be formed within an unfilled tube during the 60 casting operation are avoided, as also the excessively hard caking and fritting of the sand filling, which will occur if iron oxides are present within the bore during the operation of hot rolling, making the final removal of the sand extremely difficult, or in some cases impossible. The sand in the tube also serves to prevent the tube melting through during the steps of making the casting. 70

In the drawing, Figs. 1 and 2 are longitudinal sections of ingots cast in ingot molds. Fig. 3 is a perspective view of the drill rod and Fig. 4 is a diagrammatical view showing the rolling of the drill rod with the sand 75 core in place. In Fig. 1, 10 is the tube of mild steel with its filling of sand 11, and 12 the cast portion of the ingot cast in the ingot mold 13 from higher carbon or hard steel. The ends of tube 10 are closed by 80 screw plugs 14, and a rod 15 extends centrally through the sand 11. When this rod (elongated) is removed after the drill rod is rolled out, the removal of the sand from the bore is facilitated. 85

In Fig. 2, the tube 10' filled with sand 11 has plugs 14', 14", forced or driven in place against the compacted sand, and holes 16, 16 are made through tube and plugs, which, when the cast material 12' is poured 90 through the filling cap 17, are filled with the molten metal, making substantially cast pins 18, 18, which firmly hold the plugs 14', 14" during the operation of rolling down the drill rod, as by passing it in heated condition through rolls 19, 19, Fig. 4. The sand core is then removed from the elongated rolled down drill rod 20, leaving an open bore 21, as shown in Fig. 3. 95

I claim:

1. The process of making tubular bodies, which comprises providing a tube with bore walls substantially free of oxides, filling said tube with finely divided material, such as sand, stopping the ends of the tube with metallic stops, providing openings through the tube and extending into the metallic stops, casting an ingot about the tube utilizing the cast metal to enter the openings in the tube and stops to thereby anchor the tube 105 110

stops in place, hot rolling the ingot comprising the cast metal and included tube with the sand in the bore, and removing the sand from the elongated tubular body of reduced cross-section so produced.

2. The process of making tubular bodies, which consists in providing a tube with a core consisting of a metallic rod surrounded by sand, casting an ingot around the tube utilizing the heat of the molten material

for welding the tube in place therein and the sand for preventing the tube walls from melting through, treating the ingot and core for elongation and reduction of cross-section, and withdrawing the elongated rod and <sup>15</sup> removing the sand from the tubular body produced.

In testimony whereof, I have signed my name hereto.

PERCY A. E. ARMSTRONG.